

1

2,940,882

## MAGNETIC MATERIAL

Walter R. Hibbard, Jr., Schenectady, and John L. Walter, Scotia, N.Y., assignors to General Electric Company, a corporation of New York

No Drawing. Filed Sept. 20, 1956, Ser. No. 610,906

1 Claim. (Cl. 148—111)

This invention relates to magnetically "soft" body-centered cubic iron alloys and more particularly to a method for producing the (100) [001] crystallographic orientation with respect to the rolling plane and direction of rolling in cold-rolled and recrystallized sheet-like bodies of alloys consisting essentially of up to 5% silicon, balance substantially all iron, up to 8% aluminum, balance substantially all iron, and up to 5% molybdenum, balance substantially all iron.

As disclosed in a co-pending application for United States Letters Patent, Serial No. 610,909 filed concurrently herewith by the present inventors and assigned to the assignee of this application, sheet-like bodies composed of the previously mentioned materials have the body-centered cubic crystal lattice form and have optimum magnetic properties for certain uses when each crystal with this lattice form is oriented with respect to the rolling direction and the plane of the sheet such that the atoms which determine the planes corresponding to one pair of opposed parallel unit cube faces of the unit cube are substantially parallel to both the plane of the sheet and the rolling direction, another pair of opposed parallel unit cube faces are substantially parallel to the rolling direction and substantially perpendicular to the plane of the sheet, and the remaining pair of opposed parallel unit cube faces are substantially perpendicular to both the rolling direction and the plane of the sheet. This preferred orientation is customarily referred to as a (100) [001] orientation in the art. The numerical notation used to describe this orientation of crystal planes and directions and other crystallographic relationships which follow are according to the conventional Miller Crystallographic Index System, a more complete discussion of which may be found, for example, in "Structure of Metals," by C. S. Barrett, McGraw-Hill Book Company, Inc., New York, 2nd Edition, 1952, pages 1-25.

As more particularly set forth in our co-pending application previously referred to, polycrystalline sheet material composed of the previously described compositions having a (100) [001] "preferred orientation" may be prepared by properly rolling and appropriately heat treating grain-oriented ingots or portions thereof. It will be appreciated by those skilled in the art that the term "preferred orientation," as used herein, describes a rolled sheet metal body consisting of a plurality of grains having the body centered cubic lattice form, in which a majority of the grains, i.e., 50% or more, each have a substantially identical crystal lattice orientation with respect to the rolling direction and the plane of the sheet. The grain oriented ingots or castings from which such sheet materials have been produced have consisted primarily of a plurality of elongated columnar as-cast grains, the longitudinal axes of which are substantially parallel to each other. As disclosed in the referenced co-pending application, the desired preferred orientation is attainable in the final sheet or strip-like material by rolling the grain-oriented ingots in one or the other of two

2

alternative modes, accompanied by proper heat treatment.

We have found, however, that while the metal sheet or strip produced in accordance with the above-outlined invention invariably has the desired (100) [001] preferred orientation, otherwise known as "cube texture," that ingots having substantially identical compositions which have been cast in the same apparatus and reduced by identical processing steps resulted in grain-oriented sheet material having different degrees of grain orientation, resulting, in the cases of those materials having a lower percentage of their grains so-oriented, in materials having somewhat less desirable magnetic properties. We have discovered that the degree of preferred orientation in such sheet material is directly related to the initial orientation of the grains in the starting casting, more specifically to the angular relationship of the cube faces or (100) planes of the crystal lattices of the starting material to the rolling direction and the rolling plane during the rolling operation, and therefore by controlling this relationship, polycrystalline sheet or strip-like material having a very high degree of the desired cube texture may be invariably produced by working and recrystallizing polycrystalline grain-oriented ingots or single crystal bodies of these compositions.

It is therefore a principal object of our invention to provide a process whereby recrystallized sheet or strip-like bodies composed of silicon-iron, molybdenum-iron, and aluminum-iron alloys may be produced having a consistent high degree of cube texture preferred orientation with respect to the plane of the sheets or strips and the direction in which the sheet or strip material was rolled.

Other and specifically different objects of our invention will become apparent from the detailed disclosure and specific examples which follow.

Briefly stated and in accordance with one aspect of our invention, we have invented a process for rolling and heat-treating body-centered cubic iron base alloys to form polycrystalline sheet or strip-like material which consistently has a higher degree of cube texture grain orientation than previously attainable, by rolling said alloys so that a unit cube face of substantially every grain of said starting material is initially substantially parallel to the rolling plane and a unit cube edge of substantially every such grain is substantially parallel to the direction of rolling, and recrystallizing the so-rolled material by appropriate heat treatment.

Previous investigators have found that polycrystalline iron and body-centered cubic iron alloys such as, for example, commercial silicon-iron "electrical grade" alloys, containing about 2-5% silicon, less than about 0.005% carbon, balance substantially all iron, including minor amounts of impurities customarily present in such materials, tend to invariably assume certain well known "preferred orientations" or "texture" when subjected to substantial amounts of cold plastic deformation by unidirectional rolling. The cold-rolled texture of these materials is chiefly one in which the [110] directions of substantially all the grains lie along the direction of rolling, with a deviation of a few degrees, and (001) planes lie in the plane of the rolled sheet, with a deviation from this position chiefly about the rolling direction as an axis. These stable, cold-rolled crystal orientations have been identified as (100) [001], (115) [110], (113) [110], (112) [110], (111) [110] and (111) [112]. The higher the amount of unidirectional cold reduction given such materials, the greater is the tendency of the grains to assume a (100) [001] orientation in the rolled sheet. This may best be described as an orientation in which a pair of opposite unit cube faces of the body-centered cubic lattices of a majority of the grains in the sheet are

substantially parallel to the plane of the sheet and the remaining four unit cube faces are substantially perpendicular to the plane of the sheet and inclined at about a 45° angle to the rolling direction. Upon recrystallization by annealing such cold-rolled sheets, the preferred orientation or texture of the annealed sheet will change to an orientation which is different from the cold-rolled texture, the annealed preferred orientation of such materials has previously been found to consist of a majority of the grains having a (110) [001] orientation. This orientation may be described as one in which the unit cube lattices of the oriented grains have a plane containing diagonally oppositely cube edges substantially parallel to the plane of the sheet and a pair of opposite cube faces substantially perpendicular to the rolling direction and to the plane of the sheet. It would, therefore, reasonably be expected that when polycrystalline bodies of iron and the body-centered alloys of iron were severely cold rolled in one direction in a sheet material, the grains comprising such bodies would assume the (100) [011] stable texture or one of the previously mentioned variations thereof and when recrystallized by annealing, that the annealed texture would be predominantly the (110) [001] orientation usually obtained.

As clearly shown, however, in our previously referenced co-pending application, polycrystalline sheet or strip metal formed from cast ingots having substantially all their as-cast grains in the form of elongated columnar grains whose longitudinal axes are substantially parallel, by rolling, during which rolling the angular relationship between the longitudinal grain axes and the rolling direction and plane is maintained in one or other of the two different modes, that the resulting cold rolled material will recrystallize into a (100) [001] preferred orientation, or cube texture.

It was found upon investigation of such columnar grain-oriented ingots that the individual columnar grains all had their crystal structures oriented so that a pair of parallel unit cube faces of the body-centered cubic lattice form of the grains are substantially perpendicular to the longitudinal grain axis. However, as between individual columnar grains, the other four unit cube faces of the cubic lattice form in a particular grain were only occasionally parallel to the corresponding unit cube faces of any other grain. Since the longitudinal grain axes of the columnar grains of such an ingot are substantially parallel to each other, the unit cube faces which are substantially perpendicular to the longitudinal grain axes are substantially parallel to each other, while a similar degree of parallelism between corresponding unit cube faces which are substantially parallel to the longitudinal grain axes is found only in a few of the longitudinal grains.

We have discovered that the initial angular relationship between the unit cube faces and edges of the cubic lattices of such grains and the rolling direction and rolling plane determines the kind of orientation obtained by rolling and heat treating these materials. If the proper initial angular relationship is established and maintained during rolling, the recrystallized sheet metal resulting therefrom will consistently have a higher degree of cube texture or stated otherwise, a higher percentage of its grains will have the (100) [001] orientation than may be otherwise obtainable.

In other initial angular relationships are established and maintained during rolling, a lower percentage of cube texture will be obtained or the less desirable conventional (110) [001] preferred orientation or a variant thereof will be obtained in the recrystallized sheet material. This may best be illustrated by the following examples:

A grain-oriented ingot was prepared by casting a molten alloy consisting essentially of about 3% silicon, less than about 0.01% carbon, balance substantially all iron, into a tubular mold of fused alumina which had been preheated to about 1300° to 1400° C. and which was

provided with a bottom consisting of a water-cooled copper block which was maintained at about room temperature during the pouring and the solidification of the molten metal. During solidification, the major part of the superheat and the heat of fusion of the molten metal was extracted by means of a cooled mold bottom and the cast ingot so produced was found to be composed essentially of a plurality of elongated, columnar grains whose longitudinal axes were substantially parallel to each other and to the direction of heat extraction, as more fully discussed in our co-pending application. A slab was cut from the ingot having a pair of parallel faces extending across the width of the ingot and substantially parallel to the longitudinal axes of the columnar grains. The faces of this slab were ground to provide a slab thickness of 0.040" and then etched by means of an aqueous acid solution to a thickness of 0.032" to remove the cold worked surfaces.

The etching brought out the macrostructure of the columnar grains on the faces of the slab and the crystal orientation of a number of these grains were determined by the conventional Laue back reflection X-ray diffraction technique. After the orientation of these grains was determined, the slab was cut into two pieces along a plane perpendicular to the face of the slab and substantially parallel to the longitudinal axes of the columnar grains.

One of the slab portions containing six of the grains whose orientations had been determined and which are hereinafter identified as grains 1-6 inclusive, was cold rolled to 0.005" thick sheet material in a number of rolling passes, a cold reduction of about 84%. During this cold rolling, the longitudinal axes of the elongated columnar grains were maintained substantially parallel to the rolling direction and the slab faces were maintained parallel to the rolling plane.

The other slab portion containing three of the grains whose orientation had been determined, and which are hereinafter identified as grains 7-9 inclusive, was cold rolled to 0.011" thick sheet material in a number of rolling passes, a cold reduction of about 66%. During this cold rolling, the longitudinal axes of the elongated columnar grains were maintained substantially perpendicular to the rolling direction and the slab faces were maintained parallel to the rolling plane. The rolling was terminated at the 66% reduction in thickness because the crystals began to separate at the grain boundaries.

The nine previously identified crystals were then removed from the resulting strip by cutting along the grain boundaries with a jeweler's saw. These crystals were then etched by means of an aqueous acid solution to about 0.002" thickness and annealed at about 1000° C. for 16 hours to effect complete recrystallization of the cold worked metal. It will be appreciated that the complete recrystallization of these materials may be accomplished by heat treatment at temperatures varying from about 800° C. to 1200° C. for periods of time as short as 1/2 hour or less depending upon the particular temperature selected.

After recrystallization, the preferred orientation of the polycrystalline sheet material resulting from 9 annealed, cold worked, single crystals or grains was determined by means of conventional X-ray diffraction techniques. The crystallographic orientation of the as-cast grains comprising specimens 1-9 were similar in that in all the grains, a (100) plane or unit cube face was substantially perpendicular to the longitudinal axis of each grain. The initial grain orientation of grains 1-9 may best be described in terms of the angular relationship between the planar faces of the grain, said faces corresponding to the original slab faces, and constituting the faces upon which the deformation was accomplished, and a cube face which is parallel to the longitudinal axis of each grain and one or more edges thereof in relationship to the rolling direction or the rolling plane. These original slab faces are

parallel to the final surfaces of the sheet material and therefore parallel to the rolling plane and the plane of the resulting sheet.

Grain 1 had such a unit cube face or (100) plane tilted 27° from a parallel relationship with the grain face, said cube face having a cube edge substantially parallel to the rolling plane but inclined about 7° from the rolling direction.

Grain 2 had such a unit cube face tilted 12° from a parallel relationship with the grain face, with one of its cube edges substantially coincident with the rolling direction.

Grain 3 had such a unit cube face tilted 29° from a parallel relationship with the grain face with one of its cube edges substantially coincident with the rolling direction.

Grain 4 had such a unit cube face tilted 22° from a parallel relationship with the grain face, with one of its cube edges substantially coincident with the rolling direction.

Grain 5 had such a unit cube face tilted about 28° from a parallel relationship with the grain face, with one of its cube edges substantially coincident with the rolling direction.

Grain 6 had such a unit cube face tilted about 39° from a parallel relationship with the grain face and a cube edge substantially coincident with the rolling direction.

Grain 7 had a cube face tilted about 9° with respect to the rolling direction and one of its cube edges substantially perpendicular to the rolling direction and parallel to the rolling plane.

Grain 8 had a unit cube face tilted about 19° with respect to the rolling direction, and one of its cube edges substantially perpendicular to the rolling direction and parallel to the rolling plane.

Grain 9 had a unit cube face tilted about 40° with respect to the rolling direction and one of its cube edges substantially perpendicular to the rolling direction and parallel to the rolling plane.

After the rolled grains had been heat treated, as previously described, it was found that the polycrystalline material formed from grains 1 and 6 had assumed a (110) [001] "cube on edge" orientation, the material from grains 2, 3, 4, 5, 7 and 8 had assumed a substantially cubic texture, i.e., (100) [001], with only minor variations therefrom, and that the material from grain 9 had retained practically the same orientation as it had initially, i.e., nearly (221) [551].

From the foregoing it may be seen that single grains or crystals of these materials worked by rolling into sheet and heat treated to effect recrystallization, assume a cube texture grain orientation provided the initial material has a unit cube face substantially parallel to the rolling plane and a unit cube edge substantially parallel to the rolling direction. As seen from the behavior of these grains, in no case where the unit cube face was 30° or more from a parallel relationship to the rolling plane, was the recrystallized orientation a cube texture. In the case of grain 1, compared, for example, to grain 3, both materials had a unit cube face similarly tilted with respect to the rolling plane yet grain 1 recrystallized in the (110) [001] cube-on-edge texture and grain 3 in the (100) [001] cube texture. This may be accounted for by the fact that while both grains had a unit cube face tilted substantially equal amounts with respect to the rolling plane, the unit cube structure of grain 1 was misoriented with respect to the rolling direction, i.e., one of the unit cube edges of said unit cube face was inclined at an angle of 7° to the rolling direction, while a corresponding unit

cube edge of grain 3 was substantially parallel to the rolling direction. Therefore, greater angular deviations than 7° may be tolerated in cases where the degree of tilt of the unit cube face is small. When the angular relationship of the unit cube face approaches 30° to the rolling plane, the unit cube edge must be substantially parallel to the rolling direction in order for the sheet material to recrystallize in a cube texture grain orientation.

It is therefore apparent that if grain-oriented ingots are provided in which the crystal lattices of the several grains are substantially parallel to each other, and the ingots in which initially a high percentage of the grains have a unit cube face inclined at an angle of less than 30° to the rolling plane and a unit cube edge of said unit cube inclined about 10° or less to the rolling direction, are cold reduced at least 40% by unidirectional rolling, that upon recrystallization substantially all the grains will assume the cube texture grain orientation. Ingots having this high degree of grain orientation may be prepared, for example, by casting molten metal on an oriented seed slab or crystal, as more particularly disclosed in the co-pending applications for United States Letters Patent Ser. No. 610,907, now abandoned, Walter and Fisher, and Ser. No. 610,908, now abandoned, Grenoble, both filed concurrently herewith and assigned to the assignee of this application. Additionally, single crystals made by any known procedure such as, for example, the procedure disclosed in detail in our previously referenced co-pending application Ser. No. 610,909, may be utilized as the initial material to be rolled according to our invention to produce the desired cube texture of polycrystalline sheet material.

While certain specific examples of our invention have been included for the purpose of completely and clearly disclosing our discoveries and invention, we do not intend our invention to be limited to such examples or limited in any way except as defined in the appended claim.

What we claim as new and desire to secure by Letters Patent of the United States is:

A method for improving the degree of preferred cube texture orientation in recrystallized rolled sheet material having body-centered cubic lattice form comprising the steps of providing an intermediate rolling blank consisting of a single crystal composed of a binary alloy selected from the group consisting essentially of up to about 5% silicon, balance substantially all iron, up to about 8% aluminum, balance substantially all iron, and up to about 5% molybdenum, balance substantially all iron, reducing the thickness of said single crystal by rolling to produce a worked sheet-like body having at least 40% cold reduction, said rolling being accomplished in a substantially unidirectional manner so that a unit cube face of the body-centered crystal lattice of a majority of the metal is maintained at an angle of not more than 30° from a parallel relationship to the rolling plane and a unit cube edge of said unit cube face is maintained at an angle of not more than 10° from a parallel relationship to the rolling direction and causing said rolled sheet-like body to recrystallize in the cube texture preferred orientation by annealing said body at a temperature from 800° C. to 1200° C. for a time sufficient to cause the complete recrystallization of said metal body.

#### 65 References Cited in the file of this patent

#### UNITED STATES PATENTS

- |           |                  |               |
|-----------|------------------|---------------|
| 2,112,084 | Frey et al ----- | Mar. 22, 1938 |
| 2,307,391 | Cole et al ----- | Jan. 5, 1943  |
| 2,700,006 | Dunn -----       | Jan. 18, 1955 |